# EUROPEAN PATENT SPECIFICATION

(11) **EP 4 108 106 B1**
(45) Date of publication and mention of the grant of the patent: **05.11.2025**
(21) Application number: 22166022.8
(22) Date of filing: 27.02.2020
(51) Int. Cl.: A24C 5/00, A24D 1/02, D21H 19/52

(54) **GRAVURE PRINTED BANDED WRAPPER PAPER**
UMHÜLLUNGSPAPIER MIT TIEFGEDRUCKTEN STREIFEN
PAPIER D'EMBALLAGE EN BANDES IMPRIMÉ PAR HÉLIOGRAVURE

(30) Priority: 01.03.2019 US 201916290327
(43) Date of publication of application: 28.12.2022
(62) Divisional of application: 20159740.8
(73) Proprietor: Altria Client Services LLC, Richmond, VA 23230 (US)
(72) Inventor: SHERWOOD, Timothy S., Midlothian,, 23113 (US); DALTON, Jonathan L., Disputanta,, 23842 (US)
(74) Representative: Richardt Patentanwälte PartG mbB

(56) References cited:
- US-A- 5 263 999
- US-A1- 2006 021 625

## Description

### BACKGROUND

As part of efforts to reduce the incidence of accidental fires resulting from untended smoking articles, various jurisdictions have imposed, are imposing, and may impose in the future limitations on the burning characteristics of smoking articles. One measure of the tendency of a smoking article to cause ignition of an underlying substrate is the Ignition Propensity value. To meet common governmental requirements, the Ignition Propensity value, or IP value, for a smoking article should preferably be no greater than about 25%, when tested in accordance with ASTM E2187. More preferably, the IP value should be no greater than about 20%, and even more preferably no greater than about 10%. Accordingly, efforts to meet such limits are undertaken by various manufacturers of smoking articles.

### SUMMARY

According to the invention, there is provided a smoking article as defined by independent claim 1. Further advantageous features of the invention are defined by the dependent claims.
Nyffeler Urs (US 2006/021625 A1) discloses that a burn rate of a "make-your-own" cigarette is controlled by applying an add-on material such as a refined form of fibrous cellulose to the paper sleeve and/or tobacco rod wrapper that are used to form the assembled cigarette.
Baldwin Sheryl D (US 5,263,999 A) discloses controlling a burn rate of a cigarette by the use of a paper wrapper to which regions of cellulosic material are applied and bonded. The cellulosic material is applied during a manufacturing step for the base paper wrapper, either off or on-line of the paper wrapper-forming.

### BRIEF DESCRIPTION OF THE DRAWINGS

FIG. 1 is an example embodiment of a smoking article having banded wrapper paper as described herein.
FIG. 2 is a schematic view of an example embodiment of banded wrapper paper as described herein.
FIG. 3 is a schematic view of an example gravure printing process suitable for producing embodiments of banded wrapper paper as described herein.
FIG. 4 is an illustration of an example embodiment of a gravure cylinder as described herein.
FIGS. 5A, 5B, and 5C are illustrations of an example embodiment of a gravure cylinder etching process.
FIG. 6 is a schematic view of an example embodiment of banded wrapper paper as described herein.
FIG. 7 is an illustration of an example embodiment of a gravure cylinder as described herein.

### DETAILED DESCRIPTION

Referring to FIG. 1 , a smoking article 120, such as a cigarette, can comprise a tobacco rod 122 and a filter 132 attached to one end of the tobacco rod 122 with tipping paper 129. The tobacco rod 122 comprises a column of shredded tobacco ("cut filler") and a piece of banded wrapper paper 123 disposed about the column of shredded tobacco.

The tobacco rod 122 has a lightable or lit end 124 and a tipped end 130, which, in the case of non-filtered cigarettes, is referenced as the mouth end 130 of the smoking article 120. Cut filler tobacco is an industry-standard designation. In an example embodiment, the tobacco rod 122 has a generally circular cross section. In other example embodiments, the tobacco rod 122 can have an oval cross section or other non-circular shape cross section. The wrapper 123 is sealed along a longitudinal seam to form the tobacco rod 122.

The smoking article 120 has a nominal length measured from the edge 131 of the tipping paper to the lit end 124 of the tobacco rod 122 along a longitudinal axis of smoking article 120. By way of example, that nominal length may lie in the range of about 60 to about 100 mm.

As shown in FIG. 2, the banded wrapper paper 123 can include a base web 140 that may be made from flax, wood pulp, cellulose fiber, or the like. In an example embodiment, the base web 140 has a plurality of bands of fibrous crystalline cellulosic material 126 on one or both sides thereof. In an example embodiment, the bands of fibrous crystalline cellulosic material 126 are applied to a wire side of the base web 140 such that they are on the inside of the banded wrapper paper 123 when a piece of the wrapper 123 surrounds a column of shredded tobacco to form a tobacco rod 122.

In the manufacture of base web 140 suited for the construction of the various embodiments of banded wrapper paper disclosed herein, such manufacture usually will include the production of a roll of base web 140 of several feet across (usually about 3 feet to about 5 feet across or in transverse dimension), which is then slit into ribbons that are wound on bobbins. Printing operations are conducted on the rolls, but could be conducted after slitting. The bobbins themselves will have a transverse dimension equivalent to the width needed to make tobacco rods 122 or an integral number of such widths (e.g., 1, 2, or 4 of such widths). The bobbins are adapted for use with typical cigarette making machines. In an example embodiment, the banded wrapper paper has a dimension in cross-direction that takes into account the nominal circumference of the tobacco rod 122 and an overlapping seam. As a result, when the banded wrapper paper 123 is slit, the smoking article 120 formed therefrom always has a longitudinal seam with an exact overlap.

For purposes of this disclosure, "longitudinal" refers to the direction along the length of a tobacco rod 122 (e.g., along the axis 134 in FIG. 1), or along the length of a base web 140 (e.g., arrow 142 in FIGs. 2 and 6) used in the preparation of banded wrapper paper 123 that, in turn, may be used to fabricate a tobacco rod 122.

For purposes of this disclosure, "transverse" refers to the direction circumferentially around a tobacco rod 122 (see FIG. 1) or the direction perpendicular to the length of the base web 140 (e.g., arrow 144 in FIGs. 2 and 6) used in the preparation of banded wrapper paper 123 that, in turn, may be used to fabricate a tobacco rod 122.

For purposes of this disclosure, a "band" or "banded region" 126 is an area (see FIG. 2) on an underlying base web 140 to which a fibrous crystalline cellulosic slurry has been printed to form a region of fibrous crystalline cellulosic material. As used herein, the phrase "leading edge" refers to the edge 146 (see FIG. 1) of a banded region 126 that is closest to an approaching coal during smoldering of a smoking article 120 whose wrapper 123 contains the banded region 126, while the phrase "trailing edge" refers to the edge 148 of a banded region 126 that is farthest from an approaching coal during smoldering of a smoking article 120 whose wrapper 123 contains the banded region 126. As used herein, "band spacing" refers to the distance between the trailing edge 148 of one banded region 126 and the leading edge 146 of an adjacent banded region 126 on the base web 140 from which banded wrapper paper 123 is fashioned. As used herein, "phase" refers to the distance from the leading edge 146 of one banded region 126 to the leading edge 146 of an adjacent banded region 126.

In an example embodiment, the banded regions of fibrous crystalline cellulosic material 126 extend transversely across the base web 140 and are separated by regions free of added fibrous crystalline cellulosic material in the longitudinal direction 142 of the base web 140. The banded regions of fibrous crystalline cellulosic material 126 are applied to the base web 140 of the banded wrapper paper 123 to obtain satisfactory or improved Ignition Propensity ("IP") characteristics for a smoking article including a piece of the banded wrapper paper 123 and optionally to also obtain improved Self-Extinguishment ("SE") characteristics for the smoking article.

In an example embodiment, the banded regions of fibrous crystalline cellulosic material 126 are arranged on the base web 140 such that at least one banded region of fibrous crystalline cellulosic material 126 is positioned between the lit end 124 and the tipped end 130 of the tobacco rod 122 in each finished smoking article 120 that includes the banded wrapper paper 123. In an example embodiment, at least two banded regions of fibrous crystalline cellulosic material 126 are positioned between the lit end 124 and the tipped end 130 of the tobacco rod 122 in each finished smoking article 120 that includes the banded wrapper paper 123. In an example embodiment, the banded regions of fibrous crystalline cellulosic material 126 extend circumferentially around the tobacco rod at one or more longitudinally spaced locations along the axis 134 thereof.

It is noted for sake of convention that, in describing dimensions of various embodiments herein, that band or banded region "width" extends in a longitudinal direction along axis 142 of the base web 140 (see FIG. 2) or axis 134 of the tobacco rod 122, whereas a dimension in the circumferential direction will be expressed as "circumferential" or "transverse" or "in cross-direction."

In an example embodiment, where the banded regions of fibrous crystalline cellulosic material 126 extend transversely across the base web 140 (or circumferentially around a tobacco rod 122), the "width" of the banded regions of fibrous crystalline cellulosic material 126 is measured in the longitudinal direction 142 from a leading edge 146 to a trailing edge 148 thereof. In an example embodiment, the widths of the banded regions of fibrous crystalline cellulosic material 126 are each about 5 to about 9 mm (from the leading edge 146 to the trailing edge 148). In an example embodiment, the widths of the banded regions of fibrous crystalline cellulosic material 126 are each about 5.5 to about 7.5 mm. In an example embodiment, the widths of the banded regions of fibrous crystalline cellulosic material 126 are each about 6 to about 7 mm. In an example embodiment, adjacent banded regions of fibrous crystalline cellulosic material 126 are longitudinally spaced by regions of the base web 140 free of added fibrous crystalline cellulosic material by a distance of about 20 mm to about 30 mm. In an example embodiment, the phase (i.e., the spacing from the leading edge 146 of one banded region 126 to the leading edge 146 of an adjacent banded region 126) is about 25 mm or 27 mm. While the banded regions of fibrous crystalline cellulosic material 126 are depicted in this disclosure as solid bands, other configurations of the banded regions 126 on the base web 140 are within the spirit and scope of this disclosure, including, but not limited to, configurations in which the banded regions 126 have one or more areas free of added fibrous crystalline cellulosic material between the leading and trailing edges 146, 148 thereof.

The base web 140 of the banded wrapper paper 123 is permeable to air. Permeability of the base web 140 is typically identified in CORESTA units. A CORESTA unit measures paper permeability in terms of volumetric flow rate (i.e., cm³/sec) per unit area (i.e., cm²) per unit pressure drop (i.e., cm of water). In example embodiments, the base web 140 of the banded wrapper paper 123 has a permeability of at least about 20 CORESTA units and a basis weight of about 22 to 30 gram(s) per square meter in regions outside of the banded regions of fibrous crystalline cellulosic material 126. In this specification, the unit of measurement for basis weight, gram(s) per square meter, is abbreviated as "gsm". In example embodiments, the base web 140 of the banded wrapper paper 123 has a permeability of at least about 20 CORESTA units and a basis weight of about 25 to 27 gsm in regions outside of the banded regions of fibrous crystalline cellulosic material 126. In an example embodiment, the base web 140 of the wrapper 123 has a permeability greater than about 30 CORESTA in regions outside of the banded regions of fibrous crystalline cellulosic material 126. In an example embodiment, the base web 140 of the wrapper 123 has a permeability of about 33 CORESTA with a basis weight of about 25 gsm in regions outside of the banded regions of fibrous crystalline cellulosic material 126. In an example embodiment, the base web 140 of the wrapper 123 has a permeability of about 46 CORESTA with a basis weight of about 25 gsm in regions outside of the banded regions of fibrous crystalline cellulosic material 126. In an example embodiment, the base web 140 of the wrapper 123 has a permeability of about 60 CORESTA in regions outside of the banded regions of fibrous crystalline cellulosic material 126. In an example embodiment, the base web 140 of the wrapper 123 has a permeability of about 60 CORESTA with a basis weight of about 25 gsm in regions outside of the banded regions of fibrous crystalline cellulosic material 126. In an example embodiment, the base web 140 of the wrapper 123 has a permeability of about 60 CORESTA with a basis weight of about 26 gsm in regions outside of the banded regions of fibrous crystalline cellulosic material 126. In example embodiments, the base web 140 has a permeability greater than about 60 CORESTA with a basis weight of about 25 gsm or more, a permeability greater than about 80 CORESTA with a basis weight of about 25 gsm or more, or a permeability greater than about 100 CORESTA with a basis weight of about 25 gsm or more in regions outside of the banded regions of fibrous crystalline cellulosic material 126.

In example embodiments, application of the fibrous crystalline cellulosic slurry to a base web 140 and drying thereof, forms a banded region of fibrous crystalline cellulosic material 126 on the base web 140 that is effective to locally reduce the permeability of the base web 140 within the banded region 126. In example embodiments, bands of fibrous crystalline cellulosic slurry are printed on the base web 140 with a gravure roller 610 to reduce the permeability of the base web 140 within the banded regions of fibrous crystalline cellulosic material 126 to about 0 to about 12 CORESTA. In an example embodiment, the permeability of the base web 140 within the banded regions of fibrous crystalline cellulosic material 126 is 7 CORESTA or less.

In example embodiments, application of the fibrous crystalline cellulosic slurry to the base web 140 and drying thereof, forms a banded region of fibrous crystalline cellulosic material 126 on the base web 140 that is effective to locally reduce diffusivity values of the base web 140 from a diffusivity level of about 2 cm/sec or greater (for the base web 140 in regions free of added fibrous crystalline cellulosic material) to a value in the range of 0.0 to about 0.2 cm/sec as measured by a Sodim CO₂ Diffusivity Tester (purchased from Sodim SAS of France). To measure the diffusivity of a piece of banded wrapper paper 123 using a Diffusivity Tester, the banded wrapper paper 123 is positioned within a clamping head so that the banded wrapper paper 123 separates two vertically arranged chambers. The upper chamber contains a carrier gas, such as nitrogen, while the lower chamber contains a marker gas, such as carbon dioxide. There is no pressure difference between the two chambers such that there is no permeability effect, which occurs when a pressure difference is maintained between two surfaces of the banded wrapper paper 123. As such, any migration of gases between the two chambers is due to differences in concentrations of the gases. After a predetermined period of time (e.g., for about 25 seconds or less), the concentration of carbon dioxide within the nitrogen stream of the upper chamber is measured in an analyzer. A computer then converts the detected level of concentration into a measure of diffusivity. In an example embodiment, the diffusivity of the base web 140 within the banded regions of fibrous crystalline cellulosic material 126 is less than about 0.15 cm/sec. In an example embodiment, the diffusivity of the base web 140 within the banded regions of fibrous crystalline cellulosic material 126 is about 0 to about 0.1 cm/sec (e.g. about 0.01 to about 0.09 cm/sec, about 0.02 to about 0.08 cm/sec, about 0.03 to about 0.07 cm/sec or about 0.04 to about 0.06 cm/sec).

As used herein, "layer" refers to a quantity of fibrous crystalline cellulosic slurry printed on the base web 140 by a gravure roller from which banded wrapper paper 123 is fabricated. In an example embodiment, each banded region of fibrous crystalline cellulosic material 126 may be formed by gravure printing a "layer" of a fibrous crystalline cellulosic slurry on the base web 140 to reduce the permeability of the base web 140 in the corresponding banded region. In an example embodiment, the fibrous crystalline cellulosic slurry is aqueous.

To form the banded regions of fibrous crystalline cellulosic material 126, a single pass or multi-pass gravure printing process can be utilized. Alternatively, multiple pass gravure printing can be utilized. FIG. 3 is a schematic view of a single stage printing apparatus 602. With reference to the above-description for printing, a supply reel 601 supplies a blank base web 140 to a gravure printing station 602 where a banded region of fibrous crystalline cellulosic slurry is printed on the blank base web 140 by the gravure roller 610 and dried in a drier 634. In an example embodiment, the drier 634 can include at least one steam can. In an example embodiment, the drier 634 can include two steam cans wherein the base web 140 is advanced and pressed between the steam cans to reduce wrinkling of the base web 140. The dried, patterned base web 140 then advances to a collection reel 608. If desired, a wide base web 140 may be slit or divided by a slitter 635 into a plurality of narrower strips of base web that may be wound to form individual bobbins after the printing operation, where the bobbins have a width corresponding to that required for a smoking article 120. The optional slitter 635 may be used on the base web 140 as that base web 140 leaves the printing station, or the slitter and slitting operation may be conducted at a different location.

Example embodiments of gravure printing the fibrous crystalline cellulosic slurry as disclosed herein enable high-speed printing on the base web 140. For purposes of this disclosure, "high-speed" printing refers to printing processes where the base web 140 advances through the printing process at a linear speed greater than about 300 feet/min. In an example embodiment, the size of the crystalline fibers in the fibrous crystalline cellulosic slurry, and the deposition rate and viscosity of the fibrous crystalline cellulosic slurry are selected such that base web printing speeds of greater than 500 feet/minute can be achieved.

As shown in FIG. 4, the gravure cylinder (roller) 610 includes a plurality of cells 700 arranged in a pattern corresponding to a band that is to be printed on the base web 140 by the gravure roller 610. In an example embodiment, the gravure cylinder 610 includes two or more circumferentially spaced regions 701 of cells 700 wherein each region 701 of cells 700 is arranged in a pattern corresponding to a band that is to be printed on the base web 140 by the gravure roller 610. In this embodiment, adjacent regions 701 of cells 700 are circumferentially spaced by cell free surfaces 703 of the gravure roller 610 which extend a distance corresponding to the spacing between adjacent banded regions to be printed on the base web 140. In an embodiment, the pattern of cells 700 corresponding to banded regions are arranged in a chevron pattern wherein angle "A" at the tip or apex of the chevron is preferably greater than about 170 degrees. Such arrangement helps distribute stress due to shrinkage in the base web 140 upon application of the fibrous crystalline cellulosic slurry and drying, which in turn, helps alleviate the tendency of the paper to pucker or wrinkle in the course of gravure printing operations.

In an example embodiment, as shown in FIGS. 5A, 5B, and 5C, the cells of the gravure roller 610 can be formed by etching the gravure roller 610. Suitable etching processes and gravure cylinders can be obtained from Heliograph Holding GmbH. In an example embodiment, photoresist 801 is applied to a metallic surface 800, and lasers 802 are used to activate the photoresist, which serves to mask areas where walls are desired. In an example embodiment, as shown in FIG. 4, the gravure roller 610 (shown in FIG. 4 ) has a plurality of cells 700 which have a generally hexagonal shape. In an example embodiment, the cells 700 of the gravure roller 610 can have walls 702 ranging from about 12 x 10⁻⁶ m to about 80 x 10⁻⁶ m (about 12 to about 80 microns) in width between adjacent cells 700 depending on the desired final volume of each cell 700. In an example embodiment, the cells 700 of the gravure roller 610 can have walls 702 ranging from about 12 x 10⁻⁶ m to about 20 x 10⁻⁶ m (about 12 to about 20 microns) in width between adjacent cells 700. In an example embodiment, the gravure cylinder 610 can be formed such that certain cells within a region of cells are thinner than walls of other cells of the gravure roller 610. In an example embodiment, the cells 700 of the gravure roller 610 can have a generally circular shape. In an example embodiment, the depth of the cells 700 is uniform. However, in other embodiments, the depth of the cells 700 can vary.

In use, the cells 700 are filled with the fibrous crystalline cellulosic slurry such that they may print the fibrous crystalline cellulosic slurry on the base web 140. In an example embodiment, the cells 700 are sized to print dots of the fibrous crystalline cellulosic slurry which spread to form a continuous band of fibrous crystalline cellulosic material 126 on the base web 140 when the fibrous crystalline cellulosic slurry is dried. In an example embodiment, the cells 700 are sized to print dots of the fibrous crystalline cellulosic slurry to form a substantially continuous band of fibrous crystalline cellulosic material 126 on the base web 140 when the fibrous crystalline cellulosic slurry is dried. In an example embodiment, the cells 700 are sized to print small enough dots of the fibrous crystalline cellulosic slurry to form a non-continuous band of fibrous crystalline cellulosic material 126 on the base web 140 when the fibrous crystalline cellulosic slurry is dried wherein one or more areas within the non-continuous band of fibrous crystalline cellulosic material 126 are free of added fibrous crystalline cellulosic material. Adjustment of diffusivity of the banded regions of fibrous crystalline cellulosic material 126 can be facilitated by changing the size and/or number of cells 700 which apply fibrous crystalline cellulosic slurry.

In the printing station 602, a gravure roller 610 is supplied fibrous crystalline cellulosic slurry, and moves through a doctor blade 630 that extends along the length of the gravure roller 610. The doctor blade 630 is positioned so that is wipes the surface of the gravure roller 610 such that portions 703 of the gravure roller 610 that define the nominal spacing between adjacent banded regions 126 are essentially wiped clean of the fibrous crystalline cellulosic slurry, while the cells 700 of the gravure roller 610 advance toward a nip 616 of the printing station 602 full of the fibrous crystalline cellulosic slurry. The gravure roller 610 contacts one side of the base web 140 in the nip 616 between the gravure roller 610 and an impression cylinder 612 backed by backing roller 614 to print the fibrous crystalline cellulosic slurry in the cells of the gravure roller 610 on the base web 140. In an example embodiment, the fibrous crystalline cellulosic slurry is delivered from a reservoir 618 to an applicator 624 by a suitable pump 620. The fibrous crystalline cellulosic slurry is spread on the gravure roller 610 by the applicator 624. Excess fibrous crystalline cellulosic slurry accumulates in a bath 626 held by collector 627 from which excess fibrous crystalline cellulosic slurry returns via drain 628 to the reservoir 618. In an example embodiment, the fibrous crystalline cellulosic slurry is continuously circulated between the reservoir 618 and the bath 626 to prevent the solids in the fibrous crystalline cellulosic slurry from settling in the bottom of the reservoir 618 or the bottom of the bath 626. In an example embodiment, the fibrous crystalline cellulosic slurry in the reservoir 618 is continuously agitated or mixed, to prevent solids in the fibrous crystalline cellulosic slurry from settling in the bottom of the reservoir 618. In an embodiment, the fibrous crystalline cellulosic slurry printed on the base web 140 at room temperature. In an embodiment, the fibrous crystalline cellulosic slurry printed on the base web 140 at a temperature less than about 38° C.

In an example embodiment, the fibrous crystalline cellulosic slurry can be prepared by mixing fibrous crystalline cellulosic material and chalk with a sufficient amount of water to make an aqueous slurry having a composition of less than about 10% solids. In an example embodiment, the fibrous crystalline cellulosic material is insoluble in the water such that mixing the fibrous crystalline cellulosic material and chalk with the water suspends the fibrous crystalline cellulosic material and the chalk in the water to form a stable slurry. In an example embodiment, the fibrous crystalline cellulosic material is free of any modified cellulose. In an example embodiment, the fibrous crystalline cellulosic material is free of any binders. In an example embodiment, the fibrous crystalline cellulosic material is free of any binders and modified cellulose. In an example embodiment, the fibrous crystalline cellulosic material is free of any bacterial cellulose. In an example embodiment, the fibrous crystalline cellulosic material is microcrystalline cellulose and is free of any binders and modified cellulose. In an example embodiment, the fibrous crystalline cellulosic material is microcrystalline cellulose and a binder.

In an example embodiment, the fibrous crystalline cellulosic material includes microcrystalline cellulose and a binder, and is free of any modified cellulose. In an example embodiment, the fibrous crystalline cellulosic material is free of starch, guar gum, alginate, and/or cellulose derivatives. In an example embodiment, the fibrous crystalline cellulosic material is free of any film forming material. In an example embodiment, the fibrous crystalline cellulosic material includes a binder such as sodium carboxymethyl cellulose or carboxymethyl cellulose. In an example embodiment, the fibrous crystalline cellulosic material includes microcrystalline cellulose and a binder wherein the binder is less than about 9% by weight of the fibrous crystalline cellulosic material.

In an example embodiment, the fibrous crystalline cellulosic material includes AVICEL^{™} microcrystalline cellulose. In an example embodiment, the fibrous crystalline cellulosic material includes microcrystalline cellulose and a binder, and is free of any modified cellulose. In an example embodiment, the fibrous crystalline cellulosic material includes microcrystalline cellulose wherein the fibers of the microcrystalline cellulose are predominately of a size of about 200 x 10⁻⁶ m (about 200 microns) or less. In an example embodiment, the fibrous crystalline cellulosic material includes microcrystalline cellulose wherein at least 90% of the fibers of the microcrystalline cellulose have a size of about 200 x 10⁻⁶ m (about 200 microns) or less. In an example embodiment, the fibrous crystalline cellulosic material includes microcrystalline cellulose wherein the fibers of the microcrystalline cellulose are predominately of a size of about 10 x 10⁻⁶ m (about 10 microns) or more.

In an example embodiment, the fibrous crystalline cellulosic material is insoluble in room temperature water wherein the fibrous crystalline cellulosic material is mixed with room temperature water. In an embodiment, the fibrous crystalline cellulosic material is insoluble in water having a temperature less than about 38° C wherein the fibrous crystalline cellulosic material is mixed with water having a temperature less than about 38° C. In an example embodiment, the fibrous crystalline cellulosic material and chalk is mixed with non-deionized water such as tap water. In an example embodiment, the fibrous crystalline cellulosic slurry is a composition having less than about 9.5% fibrous crystalline cellulosic material and less than about 5.5% chalk. In an example embodiment, the fibrous crystalline cellulosic slurry is a composition having about 9.5% fibrous crystalline cellulosic material and about 5.5% chalk. In an example embodiment, the fibrous crystalline cellulosic slurry includes up to 9.5 weight % cellulosic fibrous crystalline material and up to 5.5 weight % chalk. In an embodiment, a room temperature viscosity of the fibrous crystalline cellulosic slurry is no greater than about 40 centipoises. In an example embodiment, a room temperature viscosity of the fibrous crystalline cellulosic slurry is between about 30 to 40 centipoises. In an embodiment, a room temperature viscosity of the fibrous crystalline cellulosic slurry is less than about 30 to 40 centipoises.

In an example embodiment, the fibrous crystalline cellulosic slurry is a composition having less than about 10% solids wherein a ratio fibrous crystalline cellulosic material to chalk in the fibrous crystalline cellulosic slurry is about 95 to 5. In an example embodiment, the fibrous crystalline cellulosic slurry is a composition having less than about 8% solids wherein a ratio fibrous crystalline cellulosic material to chalk in the fibrous crystalline cellulosic slurry is about 95 to 5. In an example embodiment, the fibrous crystalline cellulosic slurry is a composition having less than about 6% solids wherein a ratio fibrous crystalline cellulosic material to chalk in the fibrous crystalline cellulosic slurry is about 95 to 5. In an embodiment, the fibrous crystalline cellulosic slurry is a composition having less than about 5% solids wherein a ratio fibrous crystalline cellulosic material to chalk in the fibrous crystalline cellulosic slurry is about 95 to 5. In an embodiment, the fibrous crystalline cellulosic slurry is a composition having about 2% solids wherein a ratio fibrous crystalline cellulosic material to chalk in the fibrous crystalline cellulosic slurry is about 95 to 5. In an embodiment, the fibrous crystalline cellulosic slurry is a composition having less than about 10% solids wherein a ratio fibrous crystalline cellulosic material to chalk in the fibrous crystalline cellulosic slurry is about 94.5 to 5.5. In an embodiment, the fibrous crystalline cellulosic slurry is a composition having less than about 8% solids wherein a ratio fibrous crystalline cellulosic material to chalk in the fibrous crystalline cellulosic slurry is about 94.5 to 5.5. In an embodiment, the fibrous crystalline cellulosic slurry is a composition having less than about 6% solids wherein a ratio fibrous crystalline cellulosic material to chalk in the fibrous crystalline cellulosic slurry is about 94.5 to 5.5. In an embodiment, the fibrous crystalline cellulosic slurry is a composition having less than about 5% solids wherein a ratio fibrous crystalline cellulosic material to chalk in the fibrous crystalline cellulosic slurry is about 94.5 to 5.5. In an embodiment, the fibrous crystalline cellulosic slurry is a composition having about 2% solids wherein a ratio fibrous crystalline cellulosic material to chalk in the fibrous crystalline cellulosic slurry is about 94.5 to 5.5.

In an embodiment, the final fibrous crystalline cellulosic slurry can be printed as longitudinally spaced apart banded regions, as described with respect to FIG. 2, to a base web 140 used to form banded wrapper paper 123 for smoking articles wherein the base web 140 has a nominal width ranging from about 36 inches (i.e., about 920 mm) to about 60 inches at the gravure printing press. In an embodiment, the moisture content of the base web 140 at the time of gravure printing is at least 3%. In an embodiment, the base web 140 is passed through a sprayer operable to spray water on the base web 140 before gravure printing to increase the moisture level of the base web 140 to at least 3%.

In an embodiment, the fibrous crystalline cellulosic slurry can be applied to the base web 140 at a target rate of about 7.75 x 10⁻⁶ to 7.75 x 10⁻⁵ cubic meters per square meter (about 5 to 50 BCM (billion cubic microns per square inch)). In an embodiment, the fibrous crystalline cellulosic slurry can be applied to the base web 140 at a target rate of about 7.75 x 10⁻⁶ to about 5.89 x 10⁻⁵ cubic meters per square meter (about 5 BCM to about 38 BCM). Thereafter the base web 140 can be dried so that the printing solution dries. In an example embodiment, the fibrous crystalline cellulosic slurry is gravure printed on the base web 140 in a single pass to form bands of fibrous crystalline cellulosic material 126 wherein the total dry weight of the added fibrous crystalline cellulosic material of each band is up to about 2.5 gsm. In an example embodiment, the fibrous crystalline cellulosic slurry is gravure printed on the base web 140 in a single pass to form bands of fibrous crystalline cellulosic material 126 wherein the total dry weight of the added fibrous crystalline cellulosic material of each band is about 2.5 gsm. In an example embodiment, the fibrous crystalline cellulosic slurry is gravure printed on the base web 140 in multiple passes to form bands having multiple layers of fibrous crystalline cellulosic material 126 wherein the total dry weight of the added fibrous crystalline cellulosic material is up to about 2.5 gsm. In an example embodiment, the fibrous crystalline cellulosic slurry is gravure printed on the base web 140 in multiple passes to form bands having multiple layers of fibrous crystalline cellulosic material 126 wherein the total dry weight of the added fibrous crystalline cellulosic material is about 2.5 gsm. In an example embodiment wherein the fibrous crystalline cellulosic slurry is gravure printed on the base web 140 in multiple passes, the base web 140 may be passed through a drier 634, such as a heated can drier, to dry or partially dry the base web 140 between passes.

Once printed, the base web 140 can be passed through the drier 634 and advanced under tension to a slitter 635 where the nominal width of the base web can be longitudinally cut into a plurality of strips or ribbons, each strip having a width of about 27 mm (e.g., the width required to surround a conventional tobacco rod and have a longitudinal glue seam). While the base web 140 is still under tension, the plurality of strips can be simultaneously wound onto individual bobbins.

Ignition Propensity or IP is a standard test conducted as set forth in ASTM E 2187-04, "Standard Test Method for Measuring the Ignition Strength of Smoking Articles." Ignition propensity measures the probability that a smoking article, when smoldering and placed on a substrate, will generate sufficient heat to maintain smoldering of the tobacco rod. Low values for IP are desirable as such values correlate with a reduced likelihood that a smoldering smoking article, when inadvertently left unattended upon a substrate, will cause combustion in the substrate. An IP value of a smoking article should be no greater than about 25%, and preferably no greater than about 20%, and even more preferably no greater than about 10% as described in US Patent Application Publication No. 2013/0306082 published Nov. 21, 2013.

Self-Extinguishment or SE herein is a reference to smoldering characteristics of a smoking article under free burn conditions. To evaluate SE, a laboratory test is conducted at a temperature of 23° C +- 0.3° C and relative humidity of 55% +- 0.5%, both of which should be monitored by a recording hygrothermograph. Exhaust hood(s) remove combustion products formed during testing. Prior to testing, smoking articles to be tested are conditioned at 55% +-0.5% relative humidity and 23° C +- 0.3° C for 24 hours. Just prior to testing, the smoking articles are placed in glass beakers to assure free air access.

SE testing takes place within an enclosure or test box. A single port smoking machine or an electric lighter is used to ignite the smoking articles for the test. During testing, an apparatus or "angle holder" holds the smoking articles to be tested by holding an end at angles of 0° (horizontal), 45°, and/or 90° (vertical). Preferably, twenty (20) smoking articles are tested at each of the 0°, 45°, and 90° positions. If more than one apparatus is used, the apparatuses are preferably positioned such that the smoking articles face away from each other to avoid cross interference. If a smoking article goes out before the front line of the smoldering coal reaches the tipping paper, the outcome is scored as "self-extinguishment"; on the other hand, if the smoking article continues smoldering until the front line of the smoldering coal reaches the tipping paper, then the outcome is scored as "non-extinguishment". Thus, for example, an SE value of 95% indicates that 95% of the smoking articles tested exhibited self-extinguishment under free burn conditions; while an SE value of 20% indicates that only 20% of the smoking articles tested exhibited self-extinguishment under such free burn conditions.

The SE value for a smoking article should be no greater than about 80% (at horizontal orientation) and preferably no greater than about 50% and even more preferably no greater than about 25% as described in US Patent Application Publication No. 2013/0306082 published Nov. 21, 2013. It is desirable to achieve IP performance that meets and exceeds governmental requirements. Moreover, as also previously noted, that desired IP performance often adversely impacts the SE performance of the smoking article. Stated differently, while the IP performance may meet or exceed the governmental requirements, that IP performance is typically associated with a smoking article that will self-extinguish when hand held by a smoker- -an SE of 100%. Since smokers ordinarily prefer not to need to relight a smoking article, improvement of SE performance while maintaining IP performance constitutes a highly desirable feature for improved wrappers.

To improve SE performance, certain example band configurations disclosed herein are useful in constructing smoking articles having both improved SE performance and desired IP performance. For example, a band 126 configuration such as shown in FIG. 6 is capable of better sustaining smoldering during free burns, yet when placed adjacent a substrate, does not sustain smoldering. In addition, about 10% IP can be obtained for paper having diffusion ranging from about 0 to about 0.2 cm/sec, while maintaining about 18% SE, by controlling the print area and volume of fibrous crystalline cellulosic slurry printed on the base web 140.

As shown in FIG. 6 , banded wrapper paper 123 includes a base web 140 which includes a plurality of bands of fibrous crystalline cellulosic material 126 on one or both sides thereof. The bands of fibrous crystalline cellulosic material 126 are arranged on the base web 140 such that a smoking article 120 (see e.g., FIG. 1 ) including a piece of the banded wrapper paper 123 includes at least two bands of fibrous crystalline cellulosic material 126, wherein each band of fibrous crystalline cellulosic material has a first zone 202, a second zone 203, and a third zone 204 of fibrous crystalline cellulosic material wherein the amount of the fibrous cellulosic crystalline cellulosic material within each zone can be selected to control the IP performance and/or SE performance of a smoking article including the wrapper paper. The first zone 202 and the third zone 204 include about the same amount of fibrous crystalline cellulosic material on the base web 140, while the second zone 203 has about 20% to about 80% (e.g., about 25% to about 75%, about 30% to about 70%, about 35% to about 65%, about 40% to about 60%, or about 45% to about 55%) less fibrous crystalline cellulosic material on the base web 140 than the first or third zones 202, 204.

In an example embodiment, the fibrous crystalline cellulosic material of each zone is applied as a plurality of dots of fibrous crystalline cellulosic slurry arranged in a pattern, generally within the zone, to produce a banded region of fibrous crystalline cellulosic material on the base web 140. Moreover, each dot of fibrous crystalline cellulosic slurry printed in the second zone 203 has smaller dimensions than each dot of fibrous crystalline cellulosic slurry printed in the first zone 202 and the third zone 204. FIG. 7 shows an example embodiment of a patterned portion of a gravure cylinder (roller) 610 that may be used to print banded regions of fibrous crystalline cellulosic slurry to form banded regions of fibrous crystalline cellulosic material 126 which have a first zone 202, a second zone 203, and a third zone 204 of fibrous crystalline cellulosic material. The first, second, and third zones 202, 203, 204 of each banded region 126 are directly adjacent to one another such that they are not separated by a length of base web 140 that is free of added fibrous crystalline cellulosic material. As shown in FIG. 7 , the gravure roller 610 includes a plurality of cells 700 etched thereon in a pattern corresponding to the aforementioned zones 202, 203, 204 wherein the cells 700 have a generally hexagonal shape. In an example embodiment, the gravure cylinder 610 includes first and third zones 712 and a second zone 710 therebetween wherein walls 720 between adjacent cells 722 in the first and third zones 712 have a narrower width than walls 724 between adjacent cells 726 of the second zone 710. Because the walls 724 between adjacent cells 726 of the gravure cylinder 610 used to form the dots of printed slurry in the second zone 203 are thicker, less fibrous crystalline cellulosic slurry is applied by the gravure roller 610 and the dots of printed slurry tend to stay separated once printed on the base web 140. In contrast, dots of printed slurry in the first zone 202 and third zone 204 are formed by a gravure roller 610 including cells 722 having thinner walls 720 between adjacent cells 726, such that a greater amount of fibrous crystalline cellulosic slurry is applied and the dots of printed slurry tend to run together when printed on the base web 140. In an example embodiment, the walls 724 of the cells 726 may be configured such that the dots of printed slurry run together when printed on the base web 140. In an example embodiment, the walls 720 between adjacent cells 726 of the first and/or third zones 202, 204 may be configured such that the dots printed thereby tend to stay separated once printed on the base web 140.

The first zone 202 and the third zone 204 have a diffusivity ranging from about 0 to about 0.1 cm/sec (e.g. about 0.01 to about 0.09 cm/sec, about 0.02 to about 0.08 cm/sec, about 0.03 to about 0.07 cm/sec or about 0.04 to about 0.06 cm/sec), and the second zone 203 has a diffusivity ranging from about 0.1 to about 0.4 cm/sec (e.g. about 0.15 to about 0.35 cm/sec or about 0.2 to about 0.3 cm/sec).

When the word "about" is used in this specification in connection with a numerical value, it is intended that the associated numerical value include a tolerance of +/-10% around the stated numerical value. Moreover, when reference is made to percentages in this specification, it is intended that those percentages are based on weight, i.e., weight percentages.

The terms and phrases used herein are not to be interpreted with mathematical or geometric precision, rather geometric terminology is to be interpreted as meaning approximating or similar to the geometric terms and concepts. For example, rounded or filleted corners are intended to be included in geometric shapes such as a rectangular, hexagonal, and the like. Terms such as "generally" and "substantially" are intended to encompass both precise meanings of the associated terms and concepts as well as to provide reasonable latitude which is consistent with form, function, and/or meaning.

It will now be apparent to those skilled in the art that this specification describes a new, useful, and nonobvious smoking article, wrapper therefor, and process for making the wrapper and smoking article. It will also be apparent to those skilled in the art that numerous modifications, variations, substitutes, and equivalents exist for various aspects of the smoking article, wrapper and process that have been described in the detailed description above. Accordingly, it is expressly intended that all such modifications, variations, substitutions, and equivalents that fall within the scope of the invention, as defined by the appended claims, be embraced thereby.

## Claims

1. A smoking article (120), comprising:
a tobacco rod (122) including,
a column of filler, and
a wrapper (123) surrounding the column of filler, the tobacco rod having a circumferential direction (144), a longitudinal direction (142), a lit end (124), and a mouth end (132);
the wrapper including,
a base web (140) having generally parallel first and second side edges extending in the longitudinal direction and two ends extending in the circumferential direction,
the base web being around the column of filler such that the first and second side edges of the base web overlap and form a seam,
the base web having at least two circumferentially extending banded regions (126) of a fibrous crystalline cellulosic material thereon,
the at least two circumferentially extending banded regions longitudinally spaced along the base web,
the at least two circumferentially extended banded regions include a first zone (202), a second zone (203), and a third zone (204),
the first zone and the third zone include about the same amount of fibrous crystalline cellulose material,
the second zone includes less fibrous crystalline cellulosic material than the first zone or the third zone,
the fibrous crystalline cellulosic material having been gravure printed on the base web as a fibrous crystalline cellulosic slurry including water, crystalline cellulose, and chalk,
the fibrous crystalline cellulosic slurry having a solids content of about 10% or less by weight of the fibrous crystalline cellulosic slurry, and
the solids including the crystalline cellulose and chalk in a ratio of 94.5 to 5.5 to a ratio of 95 to 5.

2. The smoking article of claim 1, wherein the tobacco rod has a filter (132) at the mouth end.

3. The smoking article of claim 1, wherein the chalk is calcium carbonate.

4. The smoking article of claim 1, wherein the base web is free of added fibrous crystalline cellulosic material in regions outside of the at least two circumferentially extending banded regions of fibrous crystalline cellulosic material.

5. The smoking article of any one of claims 1-4, wherein the at least two circumferentially extending banded regions are longitudinally spaced along the base web by a distance of about 20 mm to about 30 mm.

6. The smoking article of claim 1, wherein the at least two circumferentially extending banded regions of fibrous crystalline cellulosic material are printed as a single layer.

7. The smoking article of claim 1, wherein the at least two circumferentially extending banded regions of fibrous crystalline cellulosic material are printed in at least two layers.

8. The smoking article of claim 1, wherein the base web has a permeability of greater than about 20 CORESTA and less than about 100 CORESTA in regions outside of the at least two circumferentially extending banded regions of fibrous crystalline cellulosic material and a CORESTA of 12 or less in regions within the at least two circumferentially extending banded regions of fibrous crystalline cellulosic material.

9. The smoking article of claim 1, wherein the at least two circumferentially extending banded regions of fibrous crystalline cellulosic material include microcrystalline cellulose.

10. The smoking article of claim 1, wherein the fibrous crystalline cellulosic material consists essentially of about 95% microcrystalline cellulose and about 5% chalk.

11. The smoking article of claim 1, wherein the fibrous crystalline cellulosic material includes microcrystalline cellulose, a binder, and chalk, wherein the binder is included in an amount of about 9% or less by weight of the of the microcrystalline cellulose.

12. The smoking article of claim 1, wherein the fibrous crystalline cellulosic material includes microcrystalline cellulose wherein at least 90% of the fibers of the microcrystalline cellulose have a size of about 200 microns or less.

13. The smoking article of claim 1, wherein the at least two banded regions of fibrous crystalline cellulosic material include up to about 2.5 gsm of added fibrous crystalline cellulosic material.

14. The smoking article of claim 1, wherein the Ignition Propensity of the smoking article is no greater than 25% and the Self-Extinguishment of the smoking article is no greater than 50%.

## Patentansprüche

1. Ein Rauchartikel (120), umfassend:
einen Tabakstab (122), umfassend
eine Füllgutsäule und
eine die Füllgutsäule umgebende Ummantelung (123), wobei der Tabakstab eine Umfangsrichtung (144), eine Längsrichtung (142), ein Brandende (124) und ein Mundende (132) aufweist;
wobei die Ummantelung umfasst:
ein Grundgewebe (140) mit im Allgemeinen parallelen ersten und zweiten Seitenrändern, die sich in Längsrichtung erstrecken, und zwei in Umfangsrichtung verlaufenden Enden,
wobei das Grundgewebe um die Füllgutsäule herum angeordnet ist, sodass der erste und der zweite Seitenrand des Grundgewebes überlappen und eine Naht bilden,
wobei das Grundgewebe mindestens zwei sich in Umfangsrichtung erstreckende bandförmige Bereiche (126) aus einem faserigen kristallinen zellulosischen Material aufweist,
wobei die mindestens zwei sich in Umfangsrichtung erstreckenden bandförmigen Bereiche entlang des Grundgewebes in Längsrichtung beabstandet sind,
wobei die mindestens zwei sich in Umfangsrichtung erstreckenden bandförmigen Bereiche eine erste Zone (202), eine zweite Zone (203) und eine dritte Zone (204) umfassen,
wobei die erste Zone und die dritte Zone ungefähr die gleiche Menge des faserigen kristallinen zellulosischen Materials enthalten,
wobei die zweite Zone weniger faseriges kristallines zellulosisches Material enthält als die erste Zone oder die dritte Zone,
wobei das faserige kristalline zellulosische Material durch Tiefdruck als eine faserige kristalline zellulosische Suspension, die Wasser, kristalline Zellulose und Kreide umfasst, auf das Grundgewebe aufgebracht wurde,
wobei die Suspension einen Feststoffgehalt von etwa 10 Gew.-% oder weniger aufweist, und
wobei die Feststoffe die kristalline Zellulose und die Kreide in einem Verhältnis von 94,5:5,5 bis 95:5 umfassen.

2. Der Rauchartikel nach Anspruch 1, wobei der Tabakstab an dem Mundende einen Filter (132) aufweist.

3. Der Rauchartikel nach Anspruch 1, wobei die Kreide Calciumcarbonat ist.

4. Der Rauchartikel nach Anspruch 1, wobei das Grundgewebe frei von zugesetztem faserigem kristallinem zellulosischem Material in Bereichen außerhalb der mindestens zwei sich in Umfangsrichtung erstreckenden bandförmigen Bereiche aus faserigem kristallinem zellulosischen Material ist.

5. Der Rauchartikel nach einem der Ansprüche 1 bis 4, wobei die mindestens zwei sich in Umfangsrichtung erstreckenden bandförmigen Bereiche entlang des Grundgewebes in Längsrichtung in einem Abstand von etwa 20 mm bis etwa 30 mm angeordnet sind.

6. Der Rauchartikel nach Anspruch 1, wobei die mindestens zwei sich in Umfangsrichtung erstreckenden bandförmigen Bereiche aus faserigem kristallinem zellulosischem Material als Einzelschicht gedruckt sind.

7. Der Rauchartikel nach Anspruch 1, wobei die mindestens zwei sich in Umfangsrichtung erstreckenden bandförmigen Bereiche aus faserigem kristallinem zellulosischem Material in mindestens zwei Schichten gedruckt sind.

8. Der Rauchartikel nach Anspruch 1, wobei das Grundgewebe in Bereichen außerhalb der mindestens zwei sich in Umfangsrichtung erstreckenden bandförmigen Bereiche aus faserigem kristallinem zellulosischem Material eine Permeabilität von größer als etwa 20 CORESTA und kleiner als etwa 100 CORESTA und in Bereichen innerhalb dieser bandförmigen Bereiche eine Permeabilität von 12 CORESTA oder weniger aufweist.

9. Der Rauchartikel nach Anspruch 1, wobei die mindestens zwei sich in Umfangsrichtung erstreckenden bandförmigen Bereiche aus faserigem kristallinem zellulosischem Material mikrokristalline Zellulose enthalten.

10. Der Rauchartikel nach Anspruch 1, wobei das faserige kristalline zellulosische Material im Wesentlichen aus etwa 95 % mikrokristalliner Zellulose und etwa 5 % Kreide besteht.

11. Der Rauchartikel nach Anspruch 1, wobei das faserige kristalline zellulosische Material mikrokristalline Zellulose, ein Bindemittel und Kreide umfasst, wobei das Bindemittel in einer Menge von etwa 9 Gew.-% oder weniger, bezogen auf die mikrokristalline Zellulose, enthalten ist.

12. Der Rauchartikel nach Anspruch 1, wobei das faserige kristalline zellulosische Material mikrokristalline Zellulose umfasst, bei der mindestens 90 % der Fasern der mikrokristallinen Zellulose eine Größe von etwa 200 Mikrometern oder weniger aufweisen.

13. Der Rauchartikel nach Anspruch 1, wobei die mindestens zwei bandförmigen Bereiche aus faserigem kristallinem zellulosischem Material bis zu etwa 2,5 g/m² an zusätzlich aufgebrachtem faserigem kristallinem zellulosischem Material enthalten.

14. Der Rauchartikel nach Anspruch 1, wobei die Entzündungsneigung des Rauchartikels nicht größer als 25 % und die Selbstverlöschung des Rauchartikels nicht größer als 50 % ist.

## Revendications

1. Article à fumer (120), comprenant : un bâton de tabac (122) incluant,
une colonne de charges, et
une enveloppe (123) entourant la colonne de charges, le bâton de tabac possédant une direction circonférentielle (144), une direction longitudinale (142), une extrémité allumée (124) et une extrémité buccale (132) ;
l'enveloppe incluant,
une toile de base (140) ayant des premier et deuxième bords latéraux généralement parallèles s'étendant dans la direction longitudinale et deux extrémités s'étendant dans la direction circonférentielle,
la toile de base entourant la colonne de charges de sorte que les premier et deuxième bords latéraux de la toile de base se superposent et forment un ourlet,
la toile de base ayant au moins deux régions en bandes (126) s'étendant circonférentiellement à base d'une matière cellulosique cristalline et fibreuse sur celle-ci,
les au moins deux régions en bandes s'étendant circonférentiellement étant espacées le long de la toile de base,
les au moins deux régions en bandes s'étendant circonférentiellement incluent une première zone (202), une deuxième zone (203) et une troisième zone (204),
la première zone est la troisième zone incluent environ la même quantité de matière cellulosique cristalline et fibreuse,
la deuxième zone inclut moins de matière cellulosique cristalline et fibreuse que la première zone ou la troisième zone,
la matière cellulosique cristalline et fibreuse ayant été imprimée par gravure sur la toile de base sous forme d'une boue cellulosique cristalline et fibreuse incluant de l'eau, de la cellulose cristalline et de la craie,
la boue cellulosique cristalline et fibreuse possédant une teneur en solides d'environ 10 % ou moins en poids de la boue cellulosique cristalline et fibreuse, et
les solides incluant la cellulose microcristalline et la craie dans un rapport de 94,5 à 5,5 à un rapport de 95 à 5.

2. Article à fumer selon la revendication 1, dans lequel le bâton de tabac a un filtre (132) au niveau de l'extrémité buccale.

3. Article à fumer selon la revendication 1, dans lequel la craie est du carbonate de calcium.

4. Article à fumer selon la revendication 1, dans lequel la toile de base est exempte de matière cellulosique cristalline et fibreuse ajoutée dans des régions à l'extérieur des au moins deux régions en bandes s'étendant circonférentiellement à base d'une matière cellulosique cristalline et fibreuse.

5. Article à fumer selon l'une quelconque des revendications 1 à 4, dans lequel les au moins deux régions en bandes s'étendant circonférentiellement sont espacées longitudinalement le long de la toile de base d'une distance d'environ 20 mm à environ 30 mm.

6. Article à fumer selon la revendication 1, dans lequel les au moins deux régions en bandes s'étendant circonférentiellement à base d'une matière cellulosique cristalline et fibreuse sont imprimées comme une seule couche.

7. Article à fumer selon la revendication 1, dans lequel les au moins deux régions en bandes s'étendant circonférentiellement à base d'une matière cellulosique cristalline et fibreuse sont imprimées en au moins deux couches.

8. Article à fumer selon la revendication 1, dans lequel la toile de base possède une perméabilité supérieure à environ 20 CORESTA et inférieure à environ 100 CORESTA dans des régions à l'extérieur des au moins deux régions en bandes s'étendant circonférentiellement à base d'une matière cellulosique cristalline et fibreuse et une CORESTA de 12 dans des régions à l'intérieur des au moins deux régions en bandes s'étendant circonférentiellement à base d'une matière cellulosique cristalline et fibreuse.

9. Article à fumer selon la revendication 1, dans lequel les au moins deux régions en bandes s'étendant circonférentiellement à base d'une matière cellulosique cristalline et fibreuse incluent de la cellulose microcristalline.

10. Article à fumer selon la revendication 1, dans lequel la matière cellulosique cristalline et fibreuse est constituée essentiellement d'environ 95 % de cellulose microcristalline et d'environ 5 % de craie.

11. Article à fumer selon la revendication 1, dans lequel la matière cellulosique cristalline et fibreuse inclut de la cellulose microcristalline, un liant et de la craie, dans lequel le liant est inclus dans une quantité d'environ 9 % ou moins en poids de la cellulose microcristalline.

12. Article à fumer selon la revendication 1, dans lequel la matière cellulosique cristalline et fibreuse inclut de la cellulose microcristalline dans lequel au moins 90 % des fibres de la cellulose microcristalline possèdent une taille d'environ 200 microns ou moins.

13. Article à fumer selon la revendication 1, dans lequel les au moins deux régions en bandes à base d'une matière cellulosique cristalline et fibreuse incluent jusqu'à 2,5 gsm de matière cellulosique cristalline et fibreuse ajoutée.

14. Article à fumer selon la revendication 1, dans lequel la propension à l'ignition de l'article à fumer n'est pas supérieure à 25 % et l'auto-extinction de l'article à fumer n'est pas supérieure à 50 %.
